

Oct. 6, 1942.

K. P. BILLNER

2,298,102

REINFORCED CONCRETE

Filed Oct. 15, 1941

2 Sheets-Sheet 1



Inventor

*Karl P. Billner*

*Sig. Raymond Webster*

Attorney

Oct. 6, 1942.

K. P. BILLNER

2,298,102

REINFORCED CONCRETE

Filed Oct. 15, 1941

2 Sheets-Sheet 2

Fig. 5.



Fig. 6.



Fig. 7.



Fig. 9.



Inventor

Karl P. Billner

By Raymond W. Colton

Attorney

## UNITED STATES PATENT OFFICE

2,298,102

## REINFORCED CONCRETE

Karl P. Billner, Philadelphia, Pa., assignor to  
Vacuum Concrete Inc., a corporation of Pennsylvania

Application October 15, 1941, Serial No. 415,128

15 Claims. (Cl. 72—71)

This invention relates to reinforced concrete members such as beams and slabs which are primarily designed to withstand loads applied transversely of their axes.

It has long been the dream of concrete engineers to design reinforced concrete structural members which will approach the strength and behavior of steel without greatly exceeding the weight of steel. The patented art is replete with disclosures seeking to fulfill that dream, but the various forms and arrangements of reinforcing elements directed towards this end have fallen short of the degree of success achieved by the present invention.

Reinforced concrete beams and slabs conforming to present practice are in general, extremely vulnerable to impact and they also lack any degree of resiliency even remotely approaching that of steel. These were the factors that limited the value of the concrete ships constructed during the emergency period of 1918. In accordance with this invention, larger and better concrete ships than heretofore believed to be feasible, can be constructed with sufficient speed to serve in the present crisis. And by virtue of this invention, not only are the impact and resiliency characteristics of reinforced concrete vastly improved, but many other properties of the material are enhanced, outstanding among which are the almost incredible increases achieved in the compressive unit stresses in the concrete, commonly represented by the symbol  $f_c$ .

Among the many shapes assigned to reinforcing elements in the development of this art is the helix, which, together with other reinforcing elements arranged in a particular manner, constitutes the basis of the improvements proposed herein. The use of helical reinforcing elements for concrete is in itself not new, since this expedient has been known and used for years in connection with compression members such as columns. An early example of such construction appears in the patent to Considere, No. 752,523, dated February 16, 1904, and along somewhat similar lines are the disclosures of Swensson, No. 871,076, dated November 12, 1907, and Maney, No. 2,035,662, dated March 31, 1936. Individual helices have likewise been proposed as reinforcing elements for concrete beams in the patent to Swensson, No. 871,075, dated November 12, 1907, and that to Keogan, No. 1,465,307, dated August 21, 1923. And helical interlocked reinforcing elements for beams and slabs have been proposed in the patent to Hartman, No. 1,233,053, dated July 10, 1917. But since the helices lie on

one side only of the neutral axis of the beam or slab and because of the relative positions of his other reinforcing elements, Hartman, like other prior inventors, has failed to disclose any structure which would even approach the characteristics which are inherent to the instant invention.

In accordance with the present invention, a reinforced concrete member such as a beam, slab or wall, primarily designed to withstand loads between its supports, contains a plurality of interlocked helices each of which has its axis extending substantially parallel to an axis of the member, and each of the helices has opposed portions of its periphery substantially adjacent opposite surfaces of the member. Tension means preferably extend through certain of the helices in a position adjacent to at least one surface of the reinforced concrete member, and preferably at a surface or surfaces designed to withstand tension. In the case of a wall such as that constituting a portion of a ship's hull where a reversal of stresses may be expected, tension rods may be arranged within some or all of the helices adjacent to both surfaces of the member. Whereas the concrete alone may perform the keying or interlocking function, one desirable procedure for maintaining the adjacent helices in interlocked relationship is to position them with their turns interlocking or overlapping to form eyes and then insert a keying rod through the eyes thus formed. These keying rods will ordinarily assume positions near the neutral axis or axes of the member and will serve admirably to oppose shearing forces. A further type of reinforcing element contemplated for the present construction includes rods arranged transversely of the axes of the helices, and such rods may be supported directly upon the longitudinal keying rods. One purpose of these transverse rods is to distribute stresses arising from impact and it is proposed for some applications that they be spaced more widely than the tension rods and if desired, alternately arranged on opposite sides of the keying rods. While adjacent helices may be arranged so that their convolutions merely overlap, it is proposed as an alternative that they be threaded together so that their individual convolutions become interlocked.

A further modification involves the introduction of additional helices having their axes disposed transversely with respect to the axes of the first helices, and inter-wound therewith, and with one another if desired, in such a manner that the axes of all of the helices will be in substan-

tially the same plane, or at least so that each helix will extend on opposite sides of the neutral axis of the member. Other reinforcing elements are contemplated for incorporation in this arrangement as well. And in cases where it may be desired to partially prefabricate the reinforcing matrix, some or all of the reinforcing elements may be assembled as a unit by suitable welding or other fastening means.

Whereas it is important that the peripheries of the helices assume positions substantially adjacent to the surfaces of the reinforced concrete members, it is likewise important, in some applications more than others, that all metal reinforcing members be protected from the elements. For this purpose primarily it is proposed that the helices and other reinforcing elements be entirely covered by a sufficient depth of concrete to serve this function.

By virtue of the constructions proposed herein, compressive unit stresses in the concrete of the order of 12,000 lbs. per square inch and higher have been developed in beams tested only four days after they were poured. And beams tested at a similar age have displayed unusually high resiliency and resistance to impact. Thus, the customary thickness or depth of concrete structures can be materially reduced with a corresponding saving in weight, adapting the invention for use in constructing ships, bridge decks, and innumerable other applications.

Added advantages are recognized when the products of the present invention are prepared in accordance with the vacuum processes set forth in the prior patents of the present inventor numbered 2,046,867 and 2,116,557, dated July 7, 1936, and May 10, 1938, respectively, and it is preferable, although not obligatory that the vacuum treatment be employed.

In fabricating a structural member of the type contemplated herein, the reinforcing elements will be assembled and maintained in their respective positions, whereupon the concrete will be poured into suitable forms enclosing the reinforcing elements. In this manner, the voids will be filled and the reinforcement embedded. Where the vacuum process is employed, at least some of the forms will be defined by mats of the general type described in the Billner patents referred to in the foregoing.

A more complete understanding of the proposed invention will be had upon reference to the attached drawings wherein:

Fig. 1 is a fragmentary end elevation partly in section and partly diagrammatic, of a structural member embodying the present invention;

Fig. 2 is a diagrammatic fragmentary longitudinal elevation along line 2-2 of Fig. 1;

Fig. 3 is a diagrammatic end elevation showing a modification;

Fig. 4 is an elevation similar to Fig. 2 taken along line 4-4 of Fig. 3;

Fig. 5 is a diagrammatic end elevation of another modification;

Fig. 6 is an elevation similar to Figs. 2 and 4 taken along line 6-6 of Fig. 5;

Figs. 7 and 8 are diagrammatic elevations at right angles to one another illustrating a modification; and

Fig. 9 is a sectional elevation illustrating the invention as applied to the construction of a wall forming a portion of a ship's hull.

The reinforced concrete member 16 in the form of a beam or slab depicted in Figs. 1 and 2 of the drawings comprises a body of concrete 18

(indicated in part by broken lines) embedding a plurality of helices 20. Adjacent helices are shown as arranged in merely overlapping relationship to define a row of eyes 22, adapted to receive a keying rod or shear bar 24 threaded through each row to interlock the helices. Within each of the helices of these figures, and adjacent the lower or tension surface 26 of the reinforced concrete beam, slab or other member, are located tension bars 28. It will be noted that the peripheries of the helices, while not exposed, extend to positions substantially adjacent to the surfaces of the member 16. It is for the purpose of protecting the metal reinforcing elements that the concrete portion of the member completely overlies the metal in addition to filling the voids between the various reinforcing elements, and embedding them.

Figs. 3 and 4 of the drawings show a modification which is similar to that of Figs. 1 and 2, but show in addition the use of tension rods 28 adjacent to both surfaces of the beam, slab or wall, an arrangement of particular importance in applications where there is a reversal of stress resulting in tension at both surfaces of the structural member.

The modification in Figs. 5 and 6 adds to the construction of Figs. 3 and 4, a mutually interlocked arrangement of the individual convolutions of adjacent helices, achieved by threading them together, combined with transverse reinforcing rods 32 crossing the axes of the spirals or helices 20 and intended primarily to distribute impact forces to which the structural member 35 may be subjected. As indicated in Fig. 6, these transverse rods need not be arranged as closely together as are the tension rods and they may be supported in staggered relationship on opposite sides of the keying rods 24.

In Figs. 7 and 8 of the drawings, the overlapping or interlocking helices 20 constituting a first group have been shown as mutually interlocked with a plurality of overlapping or interlocking helices 30 constituting a second group extending transversely of the first group and wound therethrough in such a way that the axes of all of the helices will lie in substantially the same plane, or at least, each of the helices will extend on both sides of the neutral axis of the structural member. The tension rods 28 to be arranged within the helices adjacent to the surfaces or surfaces under tension have been illustrated as extending through both groups of the helices. It will be understood that the two groups of helices need not be identical, since it may be desirable or necessary in some instances to use dissimilar stock, diameters, spacing and/or pitch.

In Fig. 9 the invention has been shown in its application to ship construction wherein the wall 34 represents a portion of a ship's hull and wherein the helices and other reinforcing elements are arranged in the manner appearing in Fig. 5. In such a case, it is quite important that the reinforcing metal including the helices be protected from the elements and this is accomplished by providing a wall thickness slightly exceeding the external diameter of the helices.

As already noted, one of the greatest deficiencies of the concrete ships constructed in the 1918 period was their vulnerability to impact and their low resiliency. By way of contrast to those old constructions, a beam designed in accordance with the present invention has been tested by the application of repeated blows of a 500 lb. weight dropped from heights beginning from one

foot and increasing by one foot increments until the height reached seven feet, by which time an ordinary beam similarly treated had completely failed while the beam of the present invention displayed only a slight amount of spalling outside of the helices. The beam embodying the present invention was then subjected to two additional blows with a weight of 2350 lbs. dropped from heights of three and four feet respectively. Then the beam was tested for leakage under a head of 16 feet of water with the result that only one-half pint per minute penetrated for each square foot of surface area. And this beam had been poured only four days previously, although it (as well as the beam reinforced in the conventional manner) had the benefit of the vacuum process of the prior patents referred to hereinbefore.

It will be interesting to analyze the results of a load test applied to a typical beam embodying the present invention. The beam identified as V-10 was tested with center loading and conformed to the following specifications:

$L=90$  in.  $b=13.5$  in.  $d=2.75$  in.

Helices: 6; diameter  $3\frac{1}{2}$  in.; pitch 1 in.; stock 25 diameter  $1\frac{1}{8}$  in.

Keying rods: 5; diameter  $\frac{1}{4}$  in.

Tension rods: 6; diameter  $\frac{3}{4}$  in. (100,000 Y. P.).

Concrete mix: 1:1:2 ( $\frac{3}{4}$  max.). 5 gallons per bag. 4 in. slump. High early strength cement. 30

Age of specimen: 4 days.  $n=10$  (assumed).

The results were as follows:

| P#     | M#      | $f_u$ #/sq. in. | $f_s$ #/sq. in. | $y'$ (P) |
|--------|---------|-----------------|-----------------|----------|
| 0      | 5,000   | 180             | 900             | 0.00     |
| 2,000  | 50,000  | 1,800           | 9,000           | 0.16     |
| 4,000  | 95,000  | 3,300           | 17,100          | 0.33     |
| 6,000  | 140,000 | 5,000           | 25,200          | 0.58     |
| 8,000  | 185,000 | 6,700           | 33,300          | 0.82     |
| 10,000 | 230,000 | 8,300           | 41,400          | 1.02     |
| 12,000 | 275,000 | 9,900           | 49,500          | 1.11     |
| 14,000 | 320,000 | 11,500          | 57,600          | 2.68     |
| 14,750 | 337,000 | 12,100          | 60,600          | 4.66     |

It will be understood that while true helices appear to be circular in cross-section, other sectional shapes may be substituted without departing from the present concept and it is intended that the term "helices" be construed to include such equivalent elements of other cross-sectional configuration. Since the invention is equally applicable to rectilinear or curved beams, slabs and walls, rather than phrase the claims in the alternative, a number of them have been worded to set forth a "member primarily designed to withstand loads applied transversely of its neutral axis" and thus include all structures of the type for which the invention is primarily intended. This expression is intended to apply equally to members such as slabs, beams or walls having either one or two neutral axes.

The method of constructing members of the type here under consideration involves arranging the helices so that adjacent ones are in overlapping relationship to form eyes, passing the keying elements or rods, in cases where they are to be used, through the eyes, inserting reinforcing elements through those helices designed to receive them, maintaining the parts thus assembled in their proper relative positions and surrounding them and filling their voids with concrete. A supplemental step greatly enhancing the value of the method thus far set forth involves the application of vacuum in accordance with the Billner patents cited herein, to remove water from the concrete. Where keying rods 75

are not used, the overlapping helices may be retained in their relative positions in any other suitable manner. In accordance with a modification already discussed, the overlapping helices extending in one direction may be interlocked by winding transversely extending helices therethrough in such a manner as to become interlocked therewith and with one another. And in some cases it may be preferred to mutually thread adjacent helices together. Another procedure is to rely upon the hardened concrete alone to maintain the overlapping helices in their interlocked relationship.

The scope of the invention is not to be restricted to the specific forms described and shown for purposes of illustration, beyond the limitations of the following claims.

I claim:

1. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member.

2. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, and tensile reinforcement extending through certain of said helices.

3. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, and tensile reinforcement extending through certain of said helices adjacent to at least one surface of said member.

4. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, and tensile reinforcement extending through certain of said helices adjacent opposite surfaces of said member.

5. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, adjacent helices having their turns in overlapping relationship defining eyes, and keying means extending through said eyes.

6. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, adjacent helices having their turns in overlapping relationship defining eyes, and shear rods extending through said eyes keying said helices together.

7. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, and reinforcing means extending transversely of the axes of said helices.

8. A reinforced concrete member primarily designed to withstand loads applied transversely of its neutral axis comprising a plurality of interlocked helices each having its axis extending substantially parallel to the axis of said member and having opposed portions of its periphery substantially adjacent opposite surfaces of said member, spaced reinforcing elements extending substantially parallel to the axes of said helices, and reinforcing rods differently spaced than said reinforcing elements extending transversely of the axes of said helices.

9. A reinforced concrete member primarily designed to withstand loads applied transversely of its neutral axis comprising a plurality of helices each having its axis extending substantially parallel to the axis of said member and having opposed portions of its periphery substantially adjacent opposite surfaces of said member, and a plurality of helices extending substantially perpendicularly to the first said helices and interlocked therewith.

10. A reinforced concrete member primarily designed to withstand loads applied transversely of its neutral axis comprising interlocked helices extending transversely with respect to one another and having their axes in substantially the same plane.

11. A reinforced concrete beam comprising a body of concrete embedding a plurality of interlocked helices each having its axis extending substantially parallel to the neutral axis of said beam and having opposed portions of its periphery substantially adjacent opposite surfaces of said beam, reinforcing elements extending through portions of said helices adjacent to said

surfaces and additional reinforcing elements extending through portions of said helices more remote from said surfaces.

12. A reinforced concrete slab comprising a row of interlocked helices arranged substantially throughout the width of said slab, each helix extending substantially parallel to the neutral axis of said slab and having opposed portions of its periphery substantially adjacent opposite surfaces of said member, reinforcing elements extending through portions of said helices adjacent to said surfaces and additional reinforcing elements extending through portions of said helices more remote from said surfaces.

13. A reinforced concrete wall comprising a plurality of interlocked helices each having its axis extending substantially parallel to the surfaces of said wall and having opposed portions of its periphery substantially adjacent to said surfaces, and reinforcing rods cooperating with said helices.

14. A reinforced concrete wall defining a portion of a ship's hull comprising a body of concrete embedding a plurality of helices each having its axis extending substantially parallel to the neutral axis of said wall and having opposed portions of its periphery adjacent to but entirely covered by opposite surfaces of said wall, adjacent helices having their turns overlapping to form a row of eyes, a keying rod projecting through said row of eyes, and reinforcing elements received within certain of said helices arranged near the surfaces of said wall designed to withstand tension and compression load reversals.

15. A reinforced concrete member primarily designed to withstand loads applied transversely of its neutral axis comprising a plurality of interlocked helices each having its axis extending substantially parallel to the axis of said member and having opposed portions of its periphery adjacent to but covered by opposite surfaces of said member.

KARL P. BILLNER.